

J. F. MONNOT.

METHOD OF MAKING CLAD METALS.

APPLICATION FILED APR. 2, 1910.

1,110,638.

Patented Sept. 15, 1914.



Witnesses:

Max B. A. Doring  
Paul H. Frank

Inventor  
John F. Monnot  
By his Attorney  
Marble Shaleley

# UNITED STATES PATENT OFFICE.

JOHN F. MONNOT, OF PARIS, FRANCE, ASSIGNOR TO DUPLEX METALS COMPANY, OF NEW YORK, N. Y., A CORPORATION OF NEW YORK.

## METHOD OF MAKING CLAD METALS.

1,110,638.

Specification of Letters Patent. Patented Sept. 15, 1914.

Application filed April 2, 1910. Serial No. 553,049.

To all whom it may concern:

Be it known that I, JOHN F. MONNOT, a citizen of the United States, residing at Paris, France, have invented certain Methods of Making Clad Metals, of which the following is a specification.

This invention relates to methods of making clad metals, and it comprises a process of producing clad metals wherein a coating 10 metal is fused and maintained in a molten condition beneath a fused cover of a mineral material comprising a halogen compound and while so molten is employed for coating iron or steel or other ferrous metal; all as 15 more fully hereinafter described and as claimed.

In the manufacture of coated metals comprising a steel or iron base firmly and permanently united by a true metallic union 20 with a coating of an unlike high melting metal, such as copper, it is necessary that the two metals be contacted in a clean state and with one metal molten so as to produce a wetting or absolute contact therebetween. 25 This absolute metallic contact, however, it is difficult to produce in practice, partly because of the free oxidizability of both metals and partly because of the difficulty of wholly obviating the presence of absorbed air or 30 gases which operate to space apart the metals to be united. In a prior application, Ser. No. 281,680, (renewed as application Ser. No. 545,712; Patent No. 971,136, Sept. 27, 1910) whereof the present application is a 35 continuation in part, I have pointed out sundry ways of obviating these difficulties; one such way being to perform the heating of the metal beneath a layer of a fused slag or flux which while acting as a heat-imparting or 40 conducting body in the heating prevents access of air to the hot metal and acts to shield it. By heating a billet or other body of solid iron or steel beneath such a layer of slag or flux, it may be raised to any desired tem- 45 perature and when withdrawn through the overlying fused material it emerges covered with a clinging layer of such flux which operates to shield it against contact with the atmosphere and hence against impairment 50 of the metallic surface by oxidation. Upon now dipping this flux covered billet in molten copper or other suitable molten coating metal which has been similarly heated to an appropriate and high temperature, the clinging flux layer is wiped off progressively 55

as the billet descends in the molten metal, giving an opportunity for the two metals to contact in an absolute manner without the presence of intervening air or gases or oxid. All fluxes are of course very much lighter 60 than molten copper, and other molten non-ferrous high-melting metals, and therefore such flux coatings will not follow the billet in its progress downward but are wiped off at the top surface of the molten metal, forming a floating layer of molten flux. 65

In making copper clad steel under the present invention, the molten copper is maintained at a temperature above the melting or ordinary casting temperature where- 7 in it assumes a peculiar condition which I have called, for the lack of another name, the supermolten condition, in which it displays a strong tendency to unite with iron and steel, alloying therewith and readily 75 forming coatings which are united with the base, with a union which is, or is equivalent to, a weld union. Clean steel dipped into "supermolten copper" and then withdrawn is found covered with a clinging film of copper or copper iron alloy with which a substantial coating of copper can readily be 80 united by casting thereagainst molten copper at a more convenient casting temperature. The joined metals so produced may be rolled, drawn and otherwise worked with the same facility as a billet of either metal and the union persists through the coexten- 85 sion. And the union so produced is indissoluble by the action of cleaving tools, such as a cold chisel, by heating and quenching, etc. 90

In the production of the molten bath of coating metal, it is convenient also to heat it beneath a covering layer of molten flux or 95 slag, as this is similarly operative in excluding air or gas and in preventing oxidation, giving such molten metal a metallic surface with which the dipped billet can readily contact to produce the desired type of union. On dipping a flux clad billet, the flux wiped off by the molten coating metal simply joins this floating layer. With this floating layer of flux above the coating metal, as pointed out in the said prior application, another 100 convenient result follows in that the copper 105 filmed billet as it is withdrawn from the molten coating metal and passes upward through the molten flux picks up another clinging layer of the latter which is con- 110

venient and effective in preventing contact of air with the sensitive surface of the hot 5  
filmed billet. If means were not taken to prevent contact of air with the relatively thin layer of copper upon the billet, such layer being, under the described circumstances, substantially only the thickness of molten metal which will cling capillarily, this coating would be oxidized, and so might 10  
disappear or might be so far converted into oxid as to hamper subsequent attachment of more copper to the filmed steel surface. This floating layer of molten flux above the molten coating metal has a further convenience where such metal contains volatilizable constituents such as the zinc of ordinary brass, in that it tends to prevent volatilization of such constituents and thereby by a change in the composition of such coating 15  
metal.

With any liquid maintained at a temperature below its boiling point, the amount of vaporization in a time unit is proportional to the free surface exposed and the concentration or "partial pressure" of the vapor 20  
in the space above such free surface. And if the hot liquid be covered with another and lighter immiscible liquid, as in covering hot water with oil, the amount of evaporation 25  
in a time unit may be very much lessened; this being due to the fact that no free surface can be exposed and that there is no free space into which the vapor can expand. These conditions obtain in melting and 30  
maintaining brass and similar alloys beneath a cover of molten flux; a flux being an immiscible fluid so far as melted metal is concerned. Under a coating of molten flux, zinc can be readily melted and raised nearly 35  
to its boiling point without much loss of metal. For this purpose the covering layer 40  
should be fairly deep. With such a deep layer of molten flux, on pouring molten metal therethrough the drops are cleaned 45  
of oxids, scale and other impurities, as well as of absorbed air, and reach the bottom of the container as clean-surfaced metal. In a way, the cleansing action is the same as that involved in pouring mercury through a 50  
deep layer of dilute acid. In making brass for instance the correct amount of zinc may be poured or dropped through a deep layer of molten flux in a suitable mold or crucible and then molten copper poured through 55  
such flux. The heat of the molten copper, which ordinarily volatilize a considerable amount of zinc, does not here do so, owing to the protective action of the layer of flux.

The whole operation of producing clad 60  
metals may conveniently be done under a layer of molten flux or slag, steel or iron to be coated being heated in a layer of molten flux, withdrawn therefrom, covered with a clinging layer of flux to protect it, dipped 65  
through a layer of molten flux resting on

a body of molten coating metal (such as brass which has been formed or melted under cover of such flux, as previously described) into such coating metal, withdrawn therefrom, covered or brazed with a clinging 70  
filmed layer of coating metal, covered as it passes through the flux with a jacketing layer of flux and then further treated. Such a film coated billet may, for example, next be placed in another vessel of flux and copper or brass at the ordinary casting temperature may be cast into proximity to the 75  
filmed surface. In this casting operation the relatively light flux does not interfere with the contact of metal and metal. In all these operations the molten flux is a protective material which precludes the access of air and the volatilization or oxidation of sensitive metals, but which does not preclude the ready production of a true metallic contact between metal and metal.

Broadly for the purposes above stated any molten inorganic non-metallic material will do for the flux, since all the silicates, borates and the like, are practically indifferent to 80  
ward metals of the classes herein contemplated and since they are all light bodies which readily float on molten metal. In so floating on the molten metal, they have an important advantage in the present invention in that being relatively poor conductors of heat they allow the metal thereunder to be raised to comparatively high temperatures. A crucible full of copper may for instance have the underlying copper in a supermolten condition while the top layers of slag or flux are at a temperature much below. The flux acts as a heat-retaining floating jacket. Borates, such as borax, calcium borate, and the like, silicates, such as the ordinary slags, waterglass, etc., are all suitable 85  
substances. The base in all the ordinary combinations of boric acid and silica with light metals, is not reducible by the heavy metals, so that these compounds may be 90  
used with copper and iron. Being, however, acid in their nature in a fused state, they readily dissolve the oxids of the heavy metals and this cleansing action is important 95  
in their use. For the present purposes, however, it is preferred to use another class of molten inorganic materials, namely, the halogen compounds. The halogen compounds of the light metals are all much 100  
more fusible than corresponding compounds containing oxygen, so that they allow work at a lower temperature. They are also more freely fluid than the silicates and borates. Salt (NaCl) for instance melts at 820° C., calcium chlorid at 780° C. and cuprous 105  
chlorid as low as 410° C. While calcium fluorid by itself melts at a comparatively high temperature, admixture of it with other halogen salts and with silicates and borates lowers its melting point very much.

The same is true of cryolite. The fluorine-containing halogen salts therefore, may very advantageously be used in connection with any of the silicates, or borates, or with the 5 other halogen compounds.

In the accompanying illustration I have shown more or less diagrammatically, and in central vertical section, one form of apparatus adapted for the carrying out of the 10 described process.

In the drawing, element 1 is a heating furnace, 2 is a heating bath filled with flux 3, and 4 is a similar heating vessel containing a layer of molten metal 5 covered by a 15 floating layer of flux 6. 7 is a stack carrying the waste gases from the furnace. 8 is a billet of iron or steel to be coated carried by hoisting mechanism 9 and adapted to be moved from place to place by conveyer 20 means 10. 11 is a mold shown as containing a layer of molten flux 12 and a filmed billet 8.

In the use of the described apparatus, the heat of the furnace melts and maintains the 25 flux in the first heating vessel in a molten condition. A billet is lowered into the molten material and there retained until it acquires a suitable heat, which may be red or yellow heat. In the second heating vessel 30 the flux is made molten by the heat from the furnace and metal melted thereunder. Such metal may be copper or silver, or other suitable non-ferrous high-melting coating metal, or it may be an alloy such as brass, 35 bronze, etc. This metal may be simply dropped through the layer of molten flux as pieces or chunks, which then melt in the crucible 4, under cover of the molten flux, so that the metal in melting, and thereafter, is 40 absolutely protected from contact with the atmosphere and it is clean surfaced and pure if originally so; or, if the coating metal be an alloy, such as brass, such alloy may be formed by melting its ingredients under 45 cover of the layer of molten flux, as above described. A billet withdrawn from the flux is plunged down through the top layer of flux in the second crucible into the molten metal where it remains until a coating is 50 formed; which ordinarily requires but a few seconds. In passing down through the flux into the molten metal this covering layer of flux is removed and joins that in the dipping bath. After the billet has become film coated 55 it is drawn upward through the flux layer where it picks up another clinging coating to protect the delicate, newly-formed film coating. This flux-coated filmed billet may now be transported to the final coating 60 vessel, or mold 11, submerged in the flux therein contained, and molten coating metal poured against it or about it, the molten metal displacing the flux upward as it descends into the mold, or the molten metal 65 for the final coating may be placed in such

mold, and protected by a covering of flux, and then the film-coated, flux covered billet may be lowered into the mold, displacing the molten metal and causing it to fill the mold. In all these operations it is desirable 70 that the flux employed be substantially the same since obviously flux from the preliminary flux heating body is constantly passing to the dipping bath and flux from the dipping bath to the final coating bath. The flux which overflows from the final coating bath may be returned to the original flux or heating bath.

The crucibles containing the molten metal and the flux may be of any neutral indifferent material, such as ordinary graphite, or may be the special material of my Patent No. 928,470.

In my Patent No. 944,371, dated December 28, 1909 (application filed July 16, 1908) 85 I have described and claimed the forming of alloys by melting the constituents, or one or more of the constituents, thereof, under a deep layer of molten covering material, and thereby reducing loss of volatilizable constituents.

As is well known, potassium chlorid (KCl) is a substantial chemical equivalent of sodium chlorid, one of the materials above named, for use as a protecting flux, and I 95 regard the use of potassium chlorid, in lieu of sodium chlorid, for such purpose, as within my invention.

Potassium chlorid for all present purposes works like sodium chlorid but it is 100 more expensive and there is no special advantage in its use alone. In admixture with sodium chlorid, however, it produces fluxes melting at a lower temperature than either.

What I claim is:—

1. The process of protecting molten metals consisting in first reducing a suitable halogen salt to a fluid condition by heat and then reducing the metal to be protected to a fluid condition by heat beneath the surface 110 of said halogen salts.

2. The method of plating iron or steel, cast or malleable, consisting in first reducing in a suitable crucible a suitable halogen salt to a fluid state by heat, then reducing below the surface of said salt the metal or metals to form a bath to a fluid condition by heat and protecting the same beneath the surface of the halogen salt and then immersing the metal to be plated first through the halogen salt into the said metal bath, and from the metal bath through the halogen salt to the atmosphere, substantially as set forth.

3. The method of protecting molten metals consisting in first reducing a suitable chlorid to a fluid condition by heat and then reducing the metal to be protected to a fluid condition by heat beneath the surface of the said chlorid.

4. The method of protecting molten metals consisting in first reducing chlorid of sodium to a fluid condition by heat, and then reducing the metal to be protected to a fluid condition by heat beneath the surface of the said chlorid of sodium.
5. The method of producing clad metal articles which consists in maintaining a bath of molten coating metal under cover of a layer of molten flux, and then immersing the metal article to be coated through such molten flux into the molten metal therebeneath, and then withdrawing such metal article through the molten flux to the atmosphere, the film of flux adhering to the article when so withdrawn protecting the

metallic film formed on the surface of said article by contact of such surface with the molten metal, and finally casting against the surface so protected a further layer of molten coating metal and permitting the molten metal so cast to solidify against such surface, the protective film of flux on the surface against which the molten metal is so cast being displaced by the molten metal as it contacts with such surface. 20  
25

In testimony whereof I affix my signature, in the presence of two witnesses.

JOHN F. MONNOT.

Witnesses:

JACK H. BAKER,  
H. C. Coxe.